

Oct. 17, 1950

R. O. HARTMAN ET AL

2,526,132

RAIL BONDING

Filed April 11, 1944

FIG. 1.



FIG. 2.



Inventors:

ROLAND O. HARTMAN and  
JOHN S. RICHARDS, deceased,  
VERA M. RICHARDS, EXECUTRIX.

by: John E. Jackson  
Their Attorney

## UNITED STATES PATENT OFFICE

2,526,132

## RAIL BONDING

Roland O. Hartman, Berea, Ohio, and John S. Richards, deceased, late of Cleveland, Ohio, by Vera M. Richards, executrix, Cleveland, Ohio, assignors to The American Steel and Wire Company of New Jersey, a corporation of New Jersey

Application April 11, 1944, Serial No. 530,548

2 Claims. (Cl. 287—20.2)

1

This invention relates to the electrical bonding of abutting railroad rail ends by the use of an electrical conductor for spanning the space between the rail ends and some means for fastening the ends of this conductor to the sides of the rail ends. Since the rails must be bonded in the field it is desirable that the mentioned means be capable of application by readily portable equipment and long ago this requirement led to the suggestion of resorting to the exothermic welding art as a medium for providing this means.

The bonding of railroad rail ends by the exothermic welding art may be done by positioning the conductor ends adjacent the rail end sides and providing molds for confining molten metal to the conductor ends and adjacent rail sides and having sprues into which such molten metal is discharged when produced by an exothermic welding mixture reacted in crucibles positioned above the sprues and having teeming ports through which the molten metal falls into these sprues. Unfortunately, this practice has the disadvantages that the molten welding metal provided in this fashion by the prior art does not alloy well with the rail end sides or with the conductor ends, the resulting welds produced by such metal are prone to contain unduly large blow holes, and this is a great disadvantage, the resulting welds, which constitute bodies of metal joining the conductor ends to the rail end sides

30

In the fashion of the more usual terminals, do

not

adequately

endure

the

vibration

encountered

in

railroad

rails

and

anything

attached

to

them.

Another

fault

with

the

weld

metal

produced

by

the

prior

art

is

that

it

does

not

have

a

very

high

tensile

strength

to

resist

being

struck

by

dragging

train

equipment.

According

to

the

present

invention

the

prior

art

practice

of

exothermically

welding

electrical

conductors

to

railroad

rail

ends

may

be

followed

In

this

tabulated

data

it

will

be

noted

that

free

aluminum

is

included

in

the

case

of

those

mixtures

of

the

higher

nickel

oxide

contents.

This

is

done

because

it

aids

proper

crushing

of

the

various

alloys

to

the

degree

required

to

produce

a

mixture

having

an

adequately

small

particle

size,

the

amount

of

aluminum

required

to

react

with

the

nickel

oxide

being

so

great

that

it

would

produce

too

much

malleability

if

used

in

alloy

form

completely.

The

various

thermit

| No. | Weld Metal  |             | Thermit Mixture |                                         |                          |                             |                             |             |      |
|-----|-------------|-------------|-----------------|-----------------------------------------|--------------------------|-----------------------------|-----------------------------|-------------|------|
|     | Per Cent Cu | Per Cent Ni | Per Cent CuO    | Per Cent Ni <sub>2</sub> O <sub>3</sub> | Per Cent Ni-Al Alloy (1) | Per Cent Cu-Ni-Al Alloy (2) | Per Cent Cu-Ni-Al Alloy (3) | Per Cent Al |      |
| 1.  | 85          | 15          | 49.75           | 9.15                                    | 36.0                     | 41.1                        |                             |             |      |
| 2.  | 70          | 30          | 64.0            |                                         | 16.7                     |                             |                             |             | 10.5 |
| 3.  | 35          | 65          | 29.6            | 43.2                                    |                          |                             |                             |             | 11.7 |
| 4.  | 35          | 65          | 24.8            | 48.6                                    |                          |                             |                             |             | 14.9 |
| 5.  | 25          | 75          | 17.45           | 58.45                                   |                          |                             |                             |             | 10.5 |
|     |             |             |                 |                                         |                          |                             |                             |             | 13.6 |

Alloy (1) 60% Ni—40% Al.  
 Alloy (2) 54.4% Cu—10.9% Ni—34.7% Al.  
 Alloy (3) 25% Cu—37.5% Ni—37.5% Al.

45 In this tabulated data it will be noted that free aluminum is included in the case of those mixtures of the higher nickel oxide contents. This is done because it aids proper crushing of the various alloys to the degree required to produce a mixture having an adequately small particle size, the amount of aluminum required to react with the nickel oxide being so great that it would produce too much malleability if used in alloy form completely. The various thermit

mixtures all provide welds having the new and unexpected results previously mentioned.

A specific example of abutting rail ends bonded in the manner described is illustrated in the accompanying drawings in which:

Figure 1 is a side view; and

Figure 2 is a section taken from the line II—II in Figure 1.

More specifically, these drawings show the sides 1 of the heads of abutting rail ends with a conductor 2 of the stranded type having its ends fixed to the sides 1 by bodies 3 made of the alloy involved by the present invention and generally contoured for the purpose of deflecting dragging train equipment as is the fashion in the case 15 of the more usual type of rail bond terminal.

We claim:

1. A bond connecting adjacent track rails comprising a conductor disposed alongside the rails and across the joint therebetween and a body of weld metal exothermically fused around each end of the conductor and to one of said rails, said body being composed of from 15 to 75% nickel and the balance copper, whereby it is alloyed with the rail to an extent such that it effectively resists detachment therefrom under the vibration to which rail joints are subject in service.

2. A bond as defined by claim 1 characterized by said body being relatively free from blowholes of substantial size.

ROLAND O. HARTMAN.

VERA M. RICHARDS,

*Administratrix of the Estate of John S. Richards,  
Deceased.*

#### REFERENCES CITED

The following references are of record in the file of this patent:

#### UNITED STATES PATENTS

| Number    | Name     | Date          |
|-----------|----------|---------------|
| 538,904   | Faulkner | May 7, 1895   |
| 802,463   | Mead     | Oct. 24, 1905 |
| 1,336,475 | Mead     | Apr. 13, 1920 |
| 2,150,045 | Ahler    | Mar. 7, 1939  |
| 2,251,820 | Caldwell | Aug. 5, 1941  |
| 2,318,604 | Febrey   | May 11, 1943  |

#### OTHER REFERENCES

15 Technical Information, Monel Metal and Nickel Alloys, TA 490 .166, copy 2 (Div. 3), revised April 15, 1936.

Development and Research Dept., The International Nickel Co. Inc., 67 Wall St., New York, N. Y., Bulletin T-1.

20 Publication: Welding Handbook (1942), pub. by Amer. Welding Society, 33 W. 39th St., New York, N. Y. (Copy Div. 14.)